

Patented Sept. 5, 1922.

1,428,246

## UNITED STATES PATENT OFFICE.

PAUL HERMANN MINCK, OF PETERSDORF, GERMANY, ASSIGNOR, BY MESNE ASSIGNMENTS, TO THE CHEMICAL FOUNDATION, INC., A CORPORATION OF DELAWARE.

### PROCESS FOR PRODUCING SPUN MATERIAL RESEMBLING WOOL, COTTON, OR CHAPPE FROM VISCOSE SOLUTIONS.

No Drawing.

Application filed May 16, 1919. Serial No. 297,712.

(GRANTED UNDER THE PROVISIONS OF THE ACT OF MARCH 3, 1921, 41 STAT. L., 1313.)

*To all whom it may concern:*

Be it known that I, PAUL HERMANN MINCK, a citizen of the free city of Hamburg, residing at Petersdorf, Riesengebirge, 5 Germany, have invented certain new and useful Improvements in Processes for Producing Spun Material Resembling Wool, Cotton, or Chappe, from Viscose Solutions (for which I have filed applications in Ger- 10 many, principal Feb. 22, 1918; 1st additional Mar. 27, 1918; 2d additional April 6, 1918; 3d additional Aug. 15, 1918; Austria, Sept. 5, 1918; Hungary, principal Dec. 5, 1918; 1st additional Dec. 5, 1918; 2d ad- 15 ditional Dec. 18, 1918), of which the following is a specification.

It is well known that in preparing viscose solutions for the manufacture of artificial silk the cellulose has to be first subjected 20 to a very thorough hydration by means of alkali lyes, as only after such treatment, it will, under action of carbon bisulphide be converted in alkaline solution into a solution sufficiently thin and homogeneous 25 so that the formation of threads which are perfectly smooth and of a high gloss, is possible.

A period from two to three days is necessary to obtain the proper degree of hydration of the cellulose, and the viscose solution prepared from such hydrated cellulose must mature for at least another four days before it may be spun. If spun immediately an absolutely dull, brittle yarn will be 35 obtained, by the highly hydrated cellulose being precipitated in the coagulating bath in a form so incapable of diffusing that the solvent agents contained in the yarn and violently decomposing therein, will likewise 40 decompose the wall of the thread.

With a continued maturation of the solution the greater part of the caustic soda and carbon bisulphide is again separated from the molecule of the cellulose alkali xan- 45 thogenate, so that it is then possible to undisturbedly precipitate the cellulose hydrate by aid of suitable precipitating baths.

The whole process is very expensive and

requires much time, as the preparation of a solution suitable for being spun into artificial silk will require about nine days, during which time certain temperatures have to be maintained, a very complicated plant is required for storing the material and lastly very complicated spinning baths 55 have to be employed in spinning the solutions. The cost of manufacture has, indeed, not played any important part in the manufacture of artificial silk, which may be considered as an article de luxe. 60

In searching to produce a wool-like spun material for which a great demand has arisen owing to the scarcity in wool and cotton the inventor proceeded from the assumption that the heretofore employed far 65 reaching hydration of the cellulose is undesirable as only the strength is required and a high gloss is of no importance if the product is to be used as a substitute for the natural fibres or for the manufacture 70 of films.

Practical research showed that there exists a suitable minimum in the hydration of the cellulose, at which the latter will, after being converted into the xanthogenate, 75 still be completely dissolved.

The novel feature of the present process consists in that a solid, soft and wool-like spun yarn is produced which may serve as a substitute for wool, cotton and chappe, 80 and yarns made therefrom, in particular such yarns which have the moderate gloss of real silk. This object is obtained by subjecting, when a viscose solution is used, the cellulose employed for such solution before 85 its treatment with carbon bisulphide and its solution, to a moderate hydration by means of caustic alkalies so that the threads will not assume the typical high gloss of artificial silk. Compared to the latter the new 90 product has the advantage of its being possible to make and spin it in a single day, whereas with the process for making artificial silk about nine days are required. Furthermore the simplest and cheapest 95 spinning baths may be employed.

The solution obtained by the new process differs from the usual viscose solutions for the manufacture of artificial silk by having a small dispersity and a comparatively 5 higher viscosity, which is about three times as high as the usual solutions.

The new spinning material which contains the cellulose in solution in a very slightly hydrated form may, contrary to 10 the known viscose solutions, be spun immediately after its production, and will yield an extremely strong and soft yarn having a soft, woollike gloss. This new result is owing to the peculiar condition of 15 these solutions. The coagulation of the threads obtained from the highly viscous solutions proceeds much more slowly, so that for this purpose spinning baths prepared from diluted mineral acids may be 20 used, without the otherwise appearing destruction of the cellulose hydrate precipitated being observed. The combination of the xanthogenate with the cellulose molecule is, owing to the moderate hydration, 25 probably weaker in the solution and the solvent agents can, in consequence of the lesser dispersity of the dissolved cellulose and the resulting higher diffusing capacity of the coagulating thread, more easily 30 emerge from the latter before the same is completely solidified.

*Example.*

100 ko. cellulose are saturated with 18% 35 soda lye and thereupon centrifuged until it contains only two parts (by weight) of lye to 1 part of cellulose. The cellulose is then left only for 12 hours approximately under the hydrating action of the alkali, 40 whereupon it is treated with 70 ko. carbon bisulphide and is dissolved in about 1600 ko. 3% soda lye. The thus obtained spinning material may be immediately spun in a 45 12-15% sulphuric acid bath, and during this spinning it is of advantage to afford the threads as long a travel through the bath as possible.

It has been further found that, particularly in well opened cellulose this already 50 greatly reduced after-hydration of the pressed out alkali cellulose by a temporary action of moderate heat and air may be entirely omitted and that in such case the yarn will become still more woollike and 55 stronger.

This represents a twofold improvement both as regards the economy of the process and the quality of the final product.

Also the solutions obtained from such 60 slightly hydrated cellulose (by a brief dipping merely) may be immediately spun in baths prepared from mineral acids and do not require a maturing period of several days. The concentration and length of 65 the spinning baths may have considerably

wider limits as the coagulating properties of the spun threads will, with decreasing hydration of the cellulose become more and more favorable.

It has been further observed that the 70 quality of the yarn is improved by reducing the quantity of carbon bisulphide coming into action and by increasing the cellulose contents of the spinning solutions. It may be here mentioned that the cellulose 75 may be dipped at the ordinary temperature, but that for the dissolution of the cellulose a somewhat lower temperature has to be maintained, which is preferably maintained at the same degree up to the spinning operation, as according to the feature of the novel process the after maturing, which is required for the production of artificial silk threads, is completely omitted.

*Example.*

85

100 ko. dry cellulose are dipped into a 17, 7% solution of caustic soda at approximately 18° cent., and left therein for about three hours. Thereupon the cellulose is 90 freed by centrifuging or pressing from the surplus soda lye until the cellulose contains not more than two parts (by weight) of lye to one part of cellulose. The thus obtained alkali cellulose is thereupon carded 95 and immediately treated with about 35% carbon bisulphide (reckoned to the dry cellulose) without exposing the latter previously to an otherwise usual maturation in closed vessels at higher temperatures. The 100 xanthogenate is then dissolved in about 1200 ko. 4% soda lye at a temperature of less than 15° cent., whereupon the solution may be immediately spun in a mineral acid bath. The solution should be stored at temperatures below 15° cent. as otherwise the 105 maturing of the viscose, which ought to be avoided, will commence.

It has been found that a very small excess of soda lye beyond two parts of the cellulose 110 weight will very unfavorably influence the quality of the viscose solution and the yarn spun therefrom.

With the present process an excess of water is to be avoided and accordingly it 115 does not depend so much on obtaining an exact percentage of caustic soda in the cellulose but on the percentage of soda lye relatively to the percentage of active water, i. e. there must be no excess of water either 120 chemically or mechanically bound by the cellulose. The smallest excess of water in the alkali cellulose will result in the xanthogenate, which is soluble in water, being prematurely dissolved, partly at least, during the treatment with carbon bisulphide, so the penetration of the but slightly hydrated cellulose fibre, which, however has already been gelatinized on its surface is impaired. The parts dissolved will in consequence of 130

the reaction heat necessarily produced by the treatment with carbon bisulphide, be decomposed or matured, which shall by all means be prevented according to my new process.

In preparing solutions for the manufacture of artificial silk this danger is of no importance, as the hydrated cellulose fibres will absorb the carbon bisulphide much 10 more readily and the spinning material produced has to subsequently mature for several days.

Experience has shown that an excess of liquid not bound by the cellulose will 15 naturally appear as soon as the cellulose contains, relatively to its weight more than a 200% aqueous solution of soda. At 200% and less the xanthogenate consists of a 20 crumbling mass, in which a gelatinization of the fibre has not yet occurred, so that the above described disadvantages as regards the solution and the spinning cannot appear.

Whereas in the manufacture of artificial 25 silk the alkali cellulose has to be subjected to storage for several days at temperatures from 20-30° cent., in order that at the further proceeding of the process the typical high gloss of the spun yarn is obtained, the 30 alkali cellulose shall, according to the present new process, even during the brief period between the dipping and the treatment with carbon bisulphide, not be subjected to temperatures higher than 20°, as 35 at higher temperatures a deeper reaching change of the cellulose molecules will immediately occur, which will affect the condition of the viscose solution and the quality of the 40 yarns spun therefrom unfavorably as regards the present process.

When the stated weight of the lye in the alkali cellulose and the temperatures are observed to which the same is exposed until it is treated with carbon bisulphide, the 45 spun material will possess the original properties of the cellulose to an almost full extent. It will combine a mild woollike gloss with a tensile strength which is 50% higher than that of the highly glossy artificial silk 50 and the considerably increased strength in a wet condition is particularly remarkable. This strength is with the new product about 55 50% of its dry strength compared to only 30% with artificial silk. The wet strength is, thus, more than 100% greater than with artificial silk.

In spinning the above described new cellulose solutions, it has been found that these 60 solutions are not always obtained of the same quality and that the yarn spun therefrom will, under circumstances be of a lesser strength. Careful investigations have shown that in such cases the cellulose employed possessed an increased oxidizing capacity, or that the soda lye was of an un-

suitable quality, containing, namely, some noxious substances, such as common salt to a high percentage.

Instead of the intended, reduced hydration of the cellulose, an oxidation of the cellulose will occur under action of the air, and this oxidation will result in a more or less weakened yarn. It is therefore necessary to obviate this danger of an oxidation.

An effective means for this has been found 75 in a comparatively small quantity of reducing substances which will not disturb the equilibrium of the solutions. Such substances are, for example, the various kinds of sugar which will burn in soda lye under 80 absorption of oxygen to carbonic acid. The oxidation threatening the cellulose will, when such means are employed, affect only the readily decomposing sugar, whilst the carbonic acid produced will serve as a further protection for the cellulose against 85 oxidizing influences.

These reducing substances may be employed in the dipping bath used for producing the alkali cellulose; when, however, 90 these baths are repeatedly used, such reducing substances will form in them by themselves having the same functions.

These means are most effective when the sulphitized cellulose is dissolved by means 95 of diluted lye, so that the reducing agents are preferably embodied in the latter. In such case a negative result is quite out of question.

As the said reducing agents are exclusively employed as means for preventing an oxidation, and shall not form a component of the finished yarn, an average of about 5% sugar will suffice, calculated to the weight of the dry cellulose. The suitable 100 quantity is determined according to the condition of the cellulose and of the soda lye.

According to the present process, therefore, reducing agents, the action of which has been accurately recognized and gauged, 110 are employed with a novel viscose solution producing a novel result, consisting in an oxidation of the cellulose being avoided and a maximum strength of the yarn produced 115 being secured.

#### Example.

100 ko. dry cellulose are hydrated in the aforesaid manner and then treated with carbon bisulphide. The xanthogenate thus 120 obtained is then dissolved in an aqueous solution of caustic soda to which about 5 ko. sugar have been added. The non-matured mass is thereupon spun in baths prepared from mineral acids.

I claim:

1. The process of producing wool-like threads from cellulose materials which comprises treating cellulose with a solution of caustic alkali sufficient to produce incom- 130

plete hydration without an excess of water, at a temperature not over 20° C., transforming the cellulose into xanthogenate by carbon bi-sulphide, dissolving the xanthogenate in an aqueous solution of caustic alkali of 3% to 5% and spinning the solution in a mineral acid bath.

2. The process of producing wool-like threads from cellulose materials which comprises dipping 100 parts of a cellulose containing material into a caustic lye of about 18% strength, at a temperature of about 18° C. allowing said cellulose containing material to remain in said lye about three hours, removing said lye from said cellulose containing material until it contains about 2 parts of lye to one part of cellulose; then treating with 35% carbon disulphide, dissolving in about 1200 parts of an aqueous solution of caustic lye at a temperature less than 15° C. and spinning in a dilute mineral acid bath.

3. The process of producing wool-like threads from cellulose materials which comprises dipping 100 parts of cellulose into a soda lye of about 18% strength at a temperature of about 18° C. allowing said cellulose to remain in said lye about three hours, removing said lye from said cellulose until it contains about 2 parts of lye to one part of cellulose; then treating with 35% carbon disulphide, dissolving in about 1200 parts of soda lye at a temperature less than 15° C. and spinning in a 12% to 15% sulphuric acid bath.

4. The process of producing wool-like threads from cellulose materials which comprises dipping 100 parts of cellulose into a soda lye of about 18% strength at a temperature of about 18° C. allowing said cellulose

to remain in said lye about three hours, removing said lye from said cellulose until it contains about two parts of lye to one part of cellulose; then treating with 35% carbon disulphide, dissolving in about 1200 parts of 4% soda lye containing a carbohydrate other than cellulose and spinning in a 12% to 15% sulphuric acid bath.

5. The process of producing wool-like threads from cellulose materials which comprises dipping 100 parts of cellulose into a soda lye of about 18% strength at a temperature of about 18° C. allowing said cellulose to remain in said lye about three hours, removing said lye from said cellulose until it contains about two parts of lye to one part of cellulose; then treating with 35% carbon disulphide, dissolving in about 1200 parts of 4% soda lye containing about 5 parts sugar and spinning in a 12% to 15% sulphuric acid bath.

6. A soft wool-like cellulose thread obtained by treating cellulose with an 18% soda lye at a temperature of about 18° C. removing said lye therefrom until there is contained therein about two parts lye to one part cellulose; then treating the 35% carbon disulphide, dissolving in 4% soda lye containing 5 parts sugar, at a temperature less than 15° and finally spinning at a 12% to 15% sulphuric acid bath, said fibres being free from a silky lustre and having a tense strength greater than that of an artificial silk thread of the same size and material.

In testimony whereof I have affixed my signature in presence of two witnesses.

PAUL HERMANN MINCK.

Witnesses:

KARL HARDIN PAUL KLUGG,  
JOHANNA MARGARETHE POLUSTINOK.